

1

3,691,033

## ADITIVE FOR TIN ELECTROPLATING

Donald Kearny Howard, Levenshulme, Manchester, Brian Martin Thomas, Woodsmoor, Stockport/Cheshire, and Alan Francis Popplewell, Didsbury, Manchester, England, and Dario Matossi, Pamplona, Spain, assignors to Ciba-Geigy Corporation

No Drawing. Filed Feb. 24, 1970, Ser. No. 13,766

Int. Cl. C23b 5/14, 5/46

U.S. Cl. 204—54 R

5 Claims 10

### ABSTRACT OF THE DISCLOSURE

The present invention provides a tin-plating additive comprising a proportion within the range of from 0.0125% to 98.7% by weight based on the total weight of the additive of 4:4'-di [dimethylamino] diphenylmethane and one or more tin-plating additives functionally active in an acidic tin-plating bath.

The present invention relates to new tin-plating additives and to tin-plating baths containing the additives.

It is known to use acidic tin-plating baths containing tin in the stannous form together with small amounts of organic additives. The incorporation of such organic additives into the tin-plating bath is made in order to increase the range of current density over which acceptable plating may be achieved. Examples of known organic tin-plating additives include condensed sulphonated phenol mixtures described and claimed in British patent specification No. 1,033,662.

However, by means of the incorporation of a tin-plating additive known for use in acidic baths or a mixture of such additives at their known working concentrations, acceptable plating is still only obtained within certain approximate limits of current density, for instance from about 60 amperes/square foot to about 450 amperes/square foot. Even at very high levels of addition, acceptable plating cannot be obtained at high current densities using known tin-plating additives alone or in admixture. In the specific case of 4:4' [dimethylamino] diphenylmethane, it is possible by the addition of very large amounts of this additive to achieve acceptable plating at very low current density but only at the expense of exceeding its solubility level in the bath and by recourse to the use of high voltages.

We have now discovered that a mixture of 4:4'-di [dimethylamino] diphenylmethane and one or more other tin-plating additives known to be functionally active in acidic tin-plating baths, when added at a similar level of concentration as conventional additives to an acidic tin-plating bath produces surprising synergistic effects resulting in satisfactory plating over a considerably wider range of current densities than can be obtained by the use of any of the additives singly or in other admixture.

Accordingly, the present invention provides a tin-plating additive comprising a proportion within the range of from 0.0125% to 98.7% by weight based on the total weight of the additive of 4:4'-di [dimethylamino] diphenylmethane and one or more tin-plating additives functionally active in an acidic tin-plating bath.

The present invention also provides a process in which a tin-plating additive is produced comprising admixing a proportion with the range of from 0.0125% to 98.7% by weight of 4:4'-di [dimethylamino] diphenylmethane and one or more tin-plating additives functionally active in acidic tin-plating baths.

Although the 4:4'-di [dimethylamino] diphenylmethane may be employed successfully in high proportions

2

in the tin-plating additive of the present invention, for optimal technical and economic advantage it is preferred not to exceed a proportion of 10% by weight. Thus, if more than 10% by weight of 4:4'-di [dimethylamino] diphenylmethane is present in the total additive, unacceptable levels of sludge-formation and/or of bath discolouration are observed in the tin-plating bath into which the tin-plating additive of the present invention is incorporated. A preferred range of proportions of 4:4'-di [dimethylamino] diphenylmethane in the total tin-plating additive is therefore from 0.0125% to 10% by weight, from 0.1% to 2.0% by weight being particularly preferred.

The second component of the tin-plating additive of the present invention may be selected from a range of additives known to be functionally active in increasing the range of current density over which acceptable plating can be achieved in conventional acidic tin-plating bath, especially the so-called "Ferrostan" bath, comprising an aqueous solution of stannous tin and phenol sulphonate acid. As examples of suitable additives there may be mentioned the sulphonated phenol additives produced according to the process described and claimed in British patent specification No. 1,033,662 that is a process comprising sulphonating phenol and/or cresol with oleum containing from 60% to 66% by weight of sulphur trioxide and thereafter heating the resulting sulphonated product for at least one hour without adding further phenol, at a subatmospheric pressure of from 5 to 25 millimeters of mercury pressure, and at a temperature in the range of from 120° to 190° C.; the phenol/polyol condensation products described in claimed in British patent specification No. 1,221,688, that is produced by reacting phenol and an aliphatic polyol containing from 2 to 8 hydroxy groups per molecule in 1:1 to 10:1 molar proportions respectively, the condensation reaction being carried out at a temperature of from 50° C. to 250° C. for a period of 1 to 10 hours; sulphonated Bisphenol A (2:2'-di-p-phenylolpropane) in acetic acid solution described and claimed in British Pat. No. 1,146,588; and an additive consisting essentially of dihydroxydiphenyl sulphone and sold under the trademark "Phenolene."

Preferably the proportion of the second tin-plating additive is within the range of from 90% to 99.9875% by weight, more preferably within the range of from 98% to 99.9% by weight of the total tin-plating additive.

According to the present invention, there is also provided an acidic tin-plating bath comprising a source of tin available for electro-plating a source of hydrogen ions and an additive comprising a proportion within the range of from 0.012% to 98.7% by weight of 4:4'-di [dimethylamino] diphenylmethane and from 99.987% to 1.3% by weight of one or more functionally-active tin-plating additives.

It is preferred to use stannous sulphate as the source of tin ions. The proportion of tin salt in the tin-plating bath is advantageously within the range of from 1.0% to 20% by weight, more preferably within the range of from 2.0% to 10% by weight, based on the total weight of the tin-plating bath.

The proportion of the tin-plating additive of the present invention in the tin-plating bath may be, for example, within the range of from 0.01% to 10% by weight, and preferably within the range of from 0.01% to 5% by weight, based on the total weight of the tin-plating bath.

In addition to the source of tin ions and the tin-plating additive of the present invention, the tin-plating bath desirably contains as the source of hydrogen ions, phenol sulphonate acid, the source of hydrogen ions preferably being present in a proportion within the range of from 0.1% to 20.0% by weight, more preferably within the range of from 0.5% to 10.0% by weight based on the total weight of the tin-plating bath.

## 3

The tin-plating additive of the present invention provides acceptable tin-plating from acidic tin-plating baths over a very wide range of current density. Moreover, the tin-plating additive of the present invention is compatible with other tin-plating bath components in all proportions which are conventionally employed for additives in acidic tin-plating baths.

The present invention is further illustrated by the fol-

## 4

relating to the plating results achieved when, as the tin-plating additive, a mixture of equal parts by weight of additives (a) and (b) listed above is employed in the standard Hull test.

As a still further comparative aid, data is presented in the table relating to the plating results achieved when only 4:4'-di [dimethylamino] diphenylmethane is employed as the tin-plating additive in the standard Hull test.

TABLE

| Example | Additives present in bath (grams/litre)                                       | Range of current density over which acceptable plating is achieved (amps./square foot) |                  |                                    |                                |
|---------|-------------------------------------------------------------------------------|----------------------------------------------------------------------------------------|------------------|------------------------------------|--------------------------------|
|         |                                                                               | Band position (cm.)                                                                    | Band width (cm.) | Actual Hull Cell current densities | Current densities <sup>1</sup> |
|         | Phenolene supra (condensation product of sulphonated o-cresol) (4.0)          | 3.3                                                                                    | 6.5              | 68-1.5                             | 450-64                         |
|         | Diphone V (sulphonated Bisphenol A derivative) (4.0)                          | 4.6                                                                                    | 4.6              | 45-2.0                             | 299-86                         |
|         | Dihydroxydiphenylsulphone (6.0)                                               | 4.3                                                                                    | 5.5              | 48-1.5                             | 330-64                         |
|         | Phenol/glucose condensation product (4.0)                                     | 4.7                                                                                    | 5.1              | 45-1.5                             | 289-64                         |
|         | Diphone V (2.0) plus phenolene supra (2.0)                                    | 4.3                                                                                    | 5.5              | 48-1.5                             | 330-64                         |
|         | Phenolene supra (4.0) plus dihydroxydiphenyl sulphone (1.0)                   | 4.1                                                                                    | 5.5              | 55-1.5                             | 350-72                         |
|         | TMADM (0.02)                                                                  | 6.5                                                                                    | 0.0              | NIL                                | NIL                            |
|         | TMADM (2.0)                                                                   | 4.0                                                                                    | 2.0              | 50-30                              | 350-260                        |
| 1       | Phenolene supra (4.0) plus TMADM (0.02)                                       | 0.2                                                                                    | 9.5              | >120-1.5                           | >700-68                        |
| 2       | Diphone V (4.0) plus TMADM (0.04)                                             | 0.4                                                                                    | 9.1              | >120-1.5                           | >700-76                        |
| 3       | Dihydroxydiphenyl sulphone (6.0) plus TMADM (0.06)                            | 0.3                                                                                    | 9.7              | >120-1.2                           | >700-55                        |
| 4       | Phenol/glucose condensation product (2.0) plus TMADM (0.02)                   | 0.5                                                                                    | 9.0              | >120-1.5                           | >700-76                        |
| 5       | Phenolene supra (4.0) plus dihydroxydiphenyl sulphone (1.0) plus TMADM (0.04) | 0.4                                                                                    | 9.1              | >120-1.7                           | >700-76                        |

<sup>1</sup> As corrected to allow for commercial plating line conditions.

Following examples. Parts and percentages shown therein are by weight unless otherwise stated. Parts by weight bear the same relation to parts by volume as do kilograms to litres.

## EXAMPLES 1 to 4

The acidic tin-plating bath solution having the following construction was made up.

55 parts by weight of an electroplating grade of stannous sulphate (to British Standard 1468:1948)  
30 parts by weight of phenol sulphonic acid  
915 parts by weight water

To this solution was added 4:4'-di [dimethylamino] diphenylmethane in conjunction with the various tin-plating additive mixtures listed below in the respective amounts per litre as given in the following table.

- (a) the commercially-available product "Phenolene Supra" ("Phenolene" is a registered trademark) which is a condensation product derived from sulphonated o-cresol produced as described in British patent specification No. 1,033,662.
- (b) the commercially-available product "Diphone V" which is believed to be a sulphonated Bisphenol A derivative and is also believed to be described and claimed in British Pat. No. 1,146,588.
- (c) the commercially-available product "Phenolene" which consists substantially of dihydroxydiphenyl sulphone. ("Phenolene" is a registered trademark).
- (d) a phenol/glucose condensation product described and claimed in our British patent specification No. 1,221,688.

250 millilitres of each of the respective solutions were placed in turn in a standard 350 millilitres Hull cell (W. Nohse, the "Hull Cell" published by R. Draper Limited, 1966) and plating was carried out at 3.0 amps at 50° C. for one minute. The results obtained are summarised in the table.

For the purpose of comparison, data are also included in the table relating to the use of the additives listed under headings (a) to (d) alone, that is, in the absence of 4:4'-di [dimethylamino] diphenylmethane (TMADM) in Hull cell tests under the standard conditions described in the previous paragraph.

As a further comparative aid, data is given in the table

What we claim is:

1. A tin electroplating additive comprising a proportion within the range of from 0.0125% to 98.7% by weight based on the total weight of additive of 4,4'-di [dimethylamino] diphenylmethane and at least one tin plating additive selected from sulphonated phenol additives produced by sulphonating phenol and/or cresol with oleum containing from 60% to 66% by weight of sulphur trioxide and thereafter heating the resulting sulphonated product for at least one hour without adding further phenol, at a subatmospheric pressure of from 5 to 25 millimeters of mercury and at a temperature in the range of from 120° C. to 190° C.; the phenol/polyol condensation products produced by reacting phenol and an aliphatic polyol containing from 2 to 8 hydroxyl groups per molecule in a 1:1 to 10:1 molar proportions respectively the condensation reaction being carried out at a temperature of from 50° C. to 250° C.; sulphonated Bisphenol A (2,2'-di-p-phenylolpropane) in acetic acid solution; and an additive consisting essentially of dihydroxydiphenyl sulphone.
2. A tin electroplating additive as claimed in claim 1 wherein the proportion of 4:4'-di [dimethylamino] diphenylmethane in the total tin-plating additive is within the range of from 0.0125% to 10% by weight.

3. A tin electroplating additive as claimed in claim 2 wherein the proportion of 4:4'- [dimethylamino] diphenylmethane in the total tin-plating additive is within the range of from 0.1% to 2.0% by weight.

4. A tin electroplating additive as claimed in claim 1 wherein the proportion of the second component is within the range of from 90% to 99.9875% by weight of the total additive.

5. A tin electroplating additive as claimed in claim 4 wherein the proportion of the second component is within the range of from 98% to 99.9% by weight of the total additive.

## References Cited

## UNITED STATES PATENTS

- |           |        |                   |           |
|-----------|--------|-------------------|-----------|
| 3,558,703 | 1/1971 | Adam et al. _____ | 260-576 X |
| 2,633,450 | 3/1953 | Andrews _____     | 204-54 R  |
| 3,515,653 | 6/1970 | Sykes _____       | 204-54 R  |

70 GERALD L. KAPLAN, Primary Examiner

U.S. Cl. X.R.